

# United States Patent [19]

Haswell, Jr. et al.

[11] Patent Number: 4,933,142

[45] Date of Patent: Jun. 12, 1990

[54] **LOW CARBON PLUS NITROGEN  
FREE-MACHINING AUSTENITIC  
STAINLESS STEELS WITH IMPROVED  
MACHINABILITY AND CORROSION  
RESISTANCE**

[75] Inventors: **Walter T. Haswell, Jr.**, Jamesville, N.Y.; **Kenneth E. Pinnow**, Pittsburgh, Pa.; **John J. Eckenrod**, Coraopolis, Pa.; **Geoffrey O. Rhodes**, Saxonburg, Pa.

[73] Assignee: **Crucible Materials Corporation**, Pittsburgh, Pa.

[21] Appl. No.: 306,216

[22] Filed: Feb. 3, 1989

## Related U.S. Application Data

[63] Continuation of Ser. No. 910,239, Sep. 19, 1986, abandoned.

[51] Int. Cl. 5 C22C 38/40; C22C 38/60

[52] U.S. Cl. 420/42; 420/49; 148/325; 148/327

[58] Field of Search 420/42, 49, 87; 148/325, 327

[56]

## References Cited

### U.S. PATENT DOCUMENTS

|           |         |                     |        |
|-----------|---------|---------------------|--------|
| 3,902,898 | 9/1975  | Denhard, Jr. et al. | 420/42 |
| 4,613,367 | 9/1986  | Eckenrod et al.     | 420/42 |
| 4,769,213 | 9/1988  | Haswell et al.      |        |
| 4,784,828 | 11/1988 | Eckenrod et al.     | 420/42 |
| 4,797,252 | 1/1989  | Eckenrod et al.     | 420/42 |

### FOREIGN PATENT DOCUMENTS

|           |        |       |        |
|-----------|--------|-------|--------|
| 48-27174  | 8/1973 | Japan | 420/49 |
| 55-122857 | 9/1980 | Japan | 420/42 |
| 61-3872   | 1/1982 | Japan | 420/49 |

### OTHER PUBLICATIONS

Lula et al., "Residual and Minor Elements in Stainless Steels", *Metallurgy of Stainless Steel*, pp. 14-1 to 14-2.

Primary Examiner—Deborah Yee  
Attorney, Agent, or Firm—Finnegan, Henderson, Farabow, Garrett & Dunner

[57]

## ABSTRACT

A low carbon plus nitrogen, free-machining, austenitic stainless steel having improved machinability and excellent corrosion resistance. The steel composition in weight percent is carbon plus nitrogen up to about 0.06, chromium 16 to 20, nickel 6 to 14, manganese up to 0.60, sulfur 0.15 to 0.50, silicon up to about 1, phosphorus up to about 0.20, molybdenum up to about 1 and balance iron.

16 Claims, No Drawings

**LOW CARBON PLUS NITROGEN  
FREE-MACHINING AUSTENITIC STAINLESS  
STEELS WITH IMPROVED MACHINABILITY  
AND CORROSION RESISTANCE**

This application is a continuation of application Ser. No. 910,239, filed Sept. 19, 1986, now abandoned.

**BACKGROUND OF THE INVENTION**

Conventional resulfurized free-machining austenitic stainless steels such as AISI Type 303 generally do not have sufficient corrosion resistance to allow them to be used in applications for acid soft drink or beverage syrups without significantly affecting the flavor of these products. The problem largely relates to the fact that the manganese or manganese-rich sulfides present in Type 303 are readily attacked in acid soft drink or beverage syrups. As a result of this attack, the local environment is so changed that the stainless steel adjacent to the manganese or manganese-rich sulfides corrodes, thereby releasing both sulfide and metal ions into the syrups and causing odor or taste problems. Passivating free-machining austenitic stainless steels such as AISI Type 303 in nitric acid solutions can minimize this difficulty by removing most of the manganese or manganese-rich sulfides from the surfaces of the articles machined from these steels before they are placed in service. However, the general corrosion resistance of the stainless steel matrix of AISI Type 303 is often insufficient, even in the absence of substantial sulfide dissolution, to avoid changes in the quality or taste of the beverage syrups. Thus, to improve the corrosion resistance of free-machining austenitic stainless steels in acid beverage syrups, the use of a more corrosion resistant free-machining additive along with improvements in the general corrosion resistance of the steel matrix in acid beverage syrups are necessary.

In this respect, U.S. Pat. No. 3,902,398 discloses that the corrosion resistance of resulfurized free-machining austenitic stainless steels can be significantly improved in acid beverage syrups by restricting their manganese content to a maximum of about 0.50% and by controlling the manganese to sulfur ratio such that chromium or chromium-rich sulfides are formed instead of manganese or manganese-rich sulfides. Chromium sulfides are more corrosion resistant than are manganese or manganese-rich sulfides in acid beverage syrups, and improve machinability but not nearly to the same extent as manganese or manganese-rich sulfides. As also disclosed in U.S. Patent 3,902,398, the loss in machinability related to the replacement of manganese or manganese-rich sulfides by chromium sulfides can be partly offset by lowering the carbon content of such steels to below about 0.035%.

In accordance with the present invention, the machinability of low-carbon resulfurized austenitic stainless steels containing chromium or chromium-rich sulfides can be substantially improved by controlling their carbon plus nitrogen content to lower than conventional levels. It has further been discovered that the addition of copper, which is known to improve the machinability of other austenitic stainless steels, not only improves the machinability of these low-manganese free-machining austenitic stainless steels, but also significantly improves their corrosion resistance in acid soft drink and beverage syrups. Thus, it is possible to substantially improve the machinability of free-machin-

ing austenitic stainless steels containing chromium or chromium-rich sulfides by lowering their carbon plus nitrogen content below conventional levels, and to further improve their machinability and especially their resistance to corrosion in acid soft drink or beverage syrups by increasing their copper content within closely controlled limits.

**OBJECTS OF THE INVENTION**

- 10 It is accordingly a primary object of the present invention to provide a chromium-nickel, free-machining austenitic stainless steel having improved machinability and high resistance to corrosion, especially in acid soft drink or beverage syrups.
- 15 An additional object of the invention is to provide a chromium-nickel-copper bearing austenitic stainless steel having improved machinability and substantially better corrosion resistance, especially in acid soft drink and beverage syrups.
- 20 Another object of this invention is to provide machined chromium-nickel austenitic stainless steel fittings and articles with improved machinability and high corrosion resistance, especially in acid soft drink and beverage syrups.
- 25 Yet another object of this invention is to provide machined chromium-nickel-copper austenitic stainless steel fittings and articles with substantially improved machinability and excellent corrosion resistance, especially in acid soft drink and beverage syrups.

**SUMMARY OF THE INVENTION**

In accordance with this invention, it has been discovered that the machinability of chromium-nickel austenitic stainless steels containing chromium or chromium-rich sulfides and with low-manganese up to 0.50% can be greatly improved by reducing their carbon plus nitrogen contents below conventional levels. In this regard, total carbon plus nitrogen in combination at low levels in accordance with the invention is more effective than either low carbon or nitrogen alone. In addition, it has been discovered that the addition of copper to these steels in controlled amounts not only improves machinability, but more importantly significantly improves their corrosion resistance, particularly in the passivated condition, in acid soft drink syrups. The improvements in machinability achieved by reducing carbon plus nitrogen content are obtained both at residual and elevated copper contents. However, the greatest improvements in machinability as well as in the resistance to corrosion in acid soft drinks are obtained with the copper bearing steels of this invention.

The steels of this invention have particular advantage in the application of fittings and articles used for handling and dispensing acid soft drink syrups. With these 55 steels, the decrease in machinability normally associated with the replacement of manganese or manganese-rich sulfides by chromium or chromium-rich sulfides is offset by the lower than conventional carbon plus nitrogen contents and by the addition of copper. Further, the copper bearing steels of this invention exhibit much better corrosion resistance in acid soft drink syrups, which is an additional advantage over prior art steels used in these applications.

In their broad composition range, the steels and machined fittings and articles of this invention consist essentially of the following elements, by weight percent:

carbon plus nitrogen—up to about 0.06%

chromium—16 to 20%  
 nickel—6 to 14%  
 manganese—up to 0.60%  
 sulfur—0.15 to 0.50%  
 phosphorus—up to 0.20%  
 silicon—up to 1%  
 molybdenum—up to 1%  
 iron—balance, except for incidental impurities

Carbon and nitrogen are normally present in the steels of this invention, but to obtain the desired improvements in machinability, it is essential in the steels of this invention to control the total carbon plus nitrogen levels below about 0.06% and preferably below about 0.05 or 0.04%.

In general, about 16 to 20% chromium and preferably 17 to 19% chromium is required in the steels of this invention to obtain the required degree of corrosion resistance in acid soft drink syrups and to adjust for the

associated with the production of stainless steels and except for up to 0.01% boron which may be added to improve hot workability.

#### DETAILED DESCRIPTION OF THE INVENTION AND SPECIFIC EXAMPLES

To demonstrate the invention and specifically the heretofore undisclosed effects of low carbon plus nitrogen and copper in accordance with the invention on machinability and corrosion resistance, fourteen 50-pound laboratory heats were vacuum induction melted and cast into ingots. The ingots were heated to 2200° F. and hot forged to 1½-inch octagonal shaped bars and air cooled. The bars in turn were annealed by heating to 1950° F., holding at 1950° F. for one hour, and then water quenching. Samples from these bars were machined to one inch square by four inch long specimens for drill machinability testing.

TABLE I

| Heat Number | Chemical Composition and Drill Machinability Rating (DMR) of Laboratory Heats |      |       |      |      |       |       |      |      |       |       |     |
|-------------|-------------------------------------------------------------------------------|------|-------|------|------|-------|-------|------|------|-------|-------|-----|
|             | Weight Percent (balance iron)                                                 |      |       |      |      |       |       |      |      |       |       |     |
|             | C                                                                             | Mn   | P     | S    | Si   | Ni    | Cr    | Mo   | Cu   | N     | C + N | DMR |
| V489        | 0.018                                                                         | 0.33 | 0.029 | 0.41 | 0.55 | 10.31 | 17.96 | 0.35 | 0.29 | 0.007 | 0.025 | 108 |
| V505        | 0.013                                                                         | 0.30 | 0.034 | 0.41 | 0.54 | 10.34 | 18.20 | 0.35 | 0.29 | 0.024 | 0.037 | 106 |
| V560        | 0.026                                                                         | 0.34 | 0.030 | 0.38 | 0.55 | 10.41 | 18.35 | 0.35 | 0.28 | 0.20  | 0.046 | 106 |
| V603        | 0.048                                                                         | 0.33 | 0.028 | 0.41 | 0.52 | 10.39 | 18.20 | 0.35 | 0.29 | 0.005 | 0.053 | 105 |
| V603A       | 0.064                                                                         | 0.34 | 0.029 | 0.41 | 0.52 | 10.42 | 18.42 | 0.35 | 0.28 | 0.010 | 0.074 | 104 |
| V506        | 0.020                                                                         | 0.30 | 0.033 | 0.39 | 0.55 | 10.37 | 18.28 | 0.35 | 0.28 | 0.059 | 0.079 | 100 |
| V541        | 0.015                                                                         | 0.35 | 0.029 | 0.39 | 0.55 | 10.13 | 18.25 | 0.35 | 0.28 | 0.091 | 0.106 | 98  |
| V563        | 0.017                                                                         | 0.35 | 0.030 | 0.39 | 0.54 | 10.39 | 18.20 | 0.35 | 0.75 | 0.016 | 0.033 | 104 |
| V508        | 0.020                                                                         | 0.33 | 0.032 | 0.39 | 0.55 | 9.31  | 18.28 | 0.35 | 1.24 | 0.029 | 0.049 | 112 |
| V507        | 0.021                                                                         | 0.32 | 0.031 | 0.39 | 0.55 | 10.48 | 18.13 | 0.35 | 1.26 | 0.023 | 0.044 | 109 |
| V564        | 0.018                                                                         | 0.36 | 0.030 | 0.40 | 0.53 | 10.29 | 18.42 | 0.34 | 1.79 | 0.021 | 0.039 | 109 |
| V567        | 0.020                                                                         | 0.59 | 0.035 | 0.42 | 0.56 | 10.84 | 18.08 | 0.35 | 2.24 | 0.012 | 0.032 | 114 |
| V568        | 0.021                                                                         | 0.57 | 0.035 | 0.41 | 0.56 | 10.64 | 18.04 | 0.73 | 2.25 | 0.023 | 0.044 | 113 |
| V565        | 0.021                                                                         | 0.34 | 0.029 | 0.36 | 0.53 | 10.35 | 18.03 | 0.34 | 2.29 | 0.025 | 0.046 | 112 |

amount of chromium involved in the formation of chromium or chromium-rich sulfides.

About 6 to 14% and preferably 8 to 11% nickel are required in the steels of this invention to obtain an austenitic microstructure and to minimize austenite transformation during processing operations at ambient temperature.

A maximum of about 0.60% manganese is required to minimize the formation of manganese or manganese-rich sulfides which are known to have an adverse effect on corrosion resistance in acid soft drink syrups and still permit the use of low cost scrap revert melting practices. In applications where maximum resistance to corrosion in acid soft drinks is required, the manganese content must be controlled below about 0.50 and the maximum manganese to sulfur ratio is 1 to 1.

A minimum of about 0.15 and a maximum of about 0.50% of sulfur are needed in the steels of this invention to obtain the desired degree of machinability.

Copper in amounts of about 0.75 to 3.00 and preferably in the amounts of 1.00 to 2.50 is very useful for increasing the stability of the austenite, for improving the machinability, and particularly for increasing the corrosion resistance of the steels of this invention in acid soft drink syrups.

Molybdenum is not necessary in the steels of this invention, but may be used in amounts up to about 1 percent for improving general corrosion resistance.

Silicon and phosphorus, may be present in amounts up to about 1% and 0.20%, respectively, in the steels of this invention. The remainder of the composition is essentially iron, except for incidental impurities usually

Table I lists the resulting chemical compositions of the laboratory heats. Other than variations in carbon, nitrogen, manganese, molybdenum and copper, all the alloys are essentially 0.40 percent sulfur, 18-percent-chromium, 10 percent nickel, free-machining austenitic stainless steels.

The machinability of the experimental alloys of Table I was evaluated using the aforementioned test specimen and a drill machinability test. In the drill machinability test, the total time taken to drill a specified number of holes to a specified depth in the material to be evaluated is compared to the total time to drill the same number of holes to the same depth in a material having known, established machining characteristics. The ratio between the time taken to drill the established material and the time taken to drill the test material multiplied by 100 provides a drill machinability rating (DMR) for the test material. Specific conditions used for these tests were as follows:

Drills—½ inch diameter high speed steel jobber bits  
 Drill Speed—405 revolutions per minute  
 Load on Drill—14.2 pounds  
 Break-in Hole Depth—0.1 inch  
 Timed Hole Depth—0.3 inch

$$\text{Drill Machinability Rating (DMR)} = \frac{\text{Time to drill established steel}}{\text{Time to drill test steel}} \times 100$$

Heat number V506 containing 0.079 percent carbon plus nitrogen, about the concentrations of these elements in a typical steel of this type, was assigned a

DMR of 100. Thus, steels having DMR values of greater than 100 have better drill machinability than conventional, typical steels of this type; and values less than 100, poorer drill machinability. Also, increasing DMR values indicate improved drill machinability.

Table I presents the results of one drill machinability testing of the laboratory steels. Allowing for some experimental scatter in the data and considering the steels containing about 0.30 percent copper and 0.025 to 0.106 percent carbon plus nitrogen, i.e., heat number V489, V505, V560, V603, V603A, V506, and V541, it is clearly evident that lowering the total combination of carbon plus nitrogen content of the steel results in improved drill machinability. Steels within the scope of the invention, i.e., heat number V489, V505, V560, and

10 15 and passivated (50% nitric acid plus 2% sodium dichromate) chips were then immersed in 50 milliliters (ml) of SPRITE syrup (pH-3) for five days. During this period of exposure, hydrogen sulfide ( $H_2S$ ) gas generation was monitored with moistened lead acetate test paper. The color changes in the lead acetate paper, if any, were recorded and rated visually in regard to the degree of  $H_2S$  evolution according to the following system: 0 —None, 1 —very light, 2 —light, 3 —moderate, 4 —heavy, 5 —very heavy. Also, at the end of the five day test period, the syrups were separated from the chips and diluted to 200 ml with deionized water. The dilute syrups were then analyzed for iron, manganese, nickel, chromium and copper ions. The results of all the soft drink syrup tests are given in Table II.

TABLE II

| Heat<br>Number | Composition |      |      |       |                     | Hydrogen Sulfide Generation and SPRITE Syrup Analysis<br>Test Results on Machined Chips |                           |                                                                       |                           |
|----------------|-------------|------|------|-------|---------------------|-----------------------------------------------------------------------------------------|---------------------------|-----------------------------------------------------------------------|---------------------------|
|                | C + N       | Mn   | S    | Ni    | Cu                  | Average Lead Acetate<br>Test Paper Rating <sup>(a)</sup>                                |                           | SPRITE Syrup Analysis<br>Total Metal Ions<br>Fe, Mn, Ni, Cr, Cu - ppm |                           |
|                |             |      |      |       |                     | As-Machined                                                                             | Passivated <sup>(b)</sup> | As-Machined                                                           | Passivated <sup>(b)</sup> |
| V505           | 0.037       | 0.30 | 0.41 | 10.34 | 0.29                | 0.1                                                                                     | 0.2                       | 78                                                                    | 57                        |
| V506           | 0.079       | 0.30 | 0.39 | 10.37 | 0.29                | 0.3                                                                                     | 0.2                       | 74                                                                    | 57                        |
| V562           | 0.033       | 0.35 | 0.39 | 10.39 | 0.75                | 0.2                                                                                     | 0.4                       | 71                                                                    | 58                        |
| V507           | 0.044       | 0.32 | 0.39 | 10.48 | 1.26                | 0                                                                                       | 0                         | 63                                                                    | 49                        |
| V508           | 0.049       | 0.33 | 0.39 | 9.31  | 1.24                | 0                                                                                       | 0                         | 63                                                                    | 45                        |
| V564           | 0.039       | 0.36 | 0.40 | 10.29 | 1.79                | 0                                                                                       | 0                         | 65                                                                    | 47                        |
| V565           | 0.046       | 0.34 | 0.36 | 10.35 | 2.29                | 0                                                                                       | 0                         | 70                                                                    | 36                        |
| A-15596        | 0.081       | 1.70 | 0.32 | 8.85  | 0.21 <sup>(c)</sup> | 5                                                                                       | 2.1                       | 330                                                                   | 120                       |

<sup>(a)</sup>Lead Acetate Test Paper Ratings = 0 - None, 1 - Very Light, 2 - Light, 3 - Moderate, 4 - Heavy, 5 - Very Heavy.

<sup>(b)</sup>Passivated (treated) in a solution of 20% nitric acid and 2% sodium dichromate for 30 minutes at 150° F.

<sup>(c)</sup>Commercial AISI Type 303 stainless.

V603, all display improved machinability compared to heat number V506.

The data in Table I also show that heat numbers V560 and V603, which have similar carbon plus nitrogen contents of about 0.05%, have similar drill machinability despite the fact that the carbon contents of the heats are respectively below and above the critical value of 0.035% specified in U.S. Patent 3,902,398 for stainless steels of this type. A like result is obtained when comparing the drill machinability of heats V506 and V603A, which have similar carbon plus nitrogen contents of about 0.075% and carbon contents respectively below and above the critical value of 0.035% specified in the above patent. Thus, carbon plus nitrogen content is more critical than carbon content in regard to the machinability of the low manganese austenitic stainless steels of this invention.

At an equivalent carbon plus nitrogen content, adding at least 1.24 percent copper to the invention steels results in still further improvements in machinability as illustrated by heat numbers V508, V507, V564, V567, and V565. A molybdenum addition to heat number V568 appears to have essentially no effect on drill machinability when compared to heat number V567 containing a similar amount of copper but less molybdenum and slightly less carbon plus nitrogen.

An empirical test in a commercial acid soft drink syrup sold under the registered tradename SPRITE was 60 conducted to compare the corrosion resistance of heat numbers V505, V506, V562, V507, V508, V564, and V565 with those disclosed in U.S. Pat. No. 3,902,348, and AISI Type 303 stainless. In this test, six-inch lengths of the bars produced from these stainless steels 65 and the AISI Type 303 were milled to the bar centers in order to obtain chips that were representative of the entire bar cross section. Ten grams of both as-machined

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8

2. The steel of claim 1 having carbon plus nitrogen up to about 0.04.
3. The steels of claim 2 having from about 0.75 copper.
4. The steels of claim 2 having 1.00 to 2.50 copper.
5. A low carbon plus nitrogen, free-machining, austenitic stainless steel having improved machinability and excellent resistance to corrosion in acid soft drink syrups, especially in the passivated condition, said steel consisting essentially of, by weight percent
- carbon plus nitrogen up to about 0.05
- chromium 17 to 19
- nickel 8 to 11
- manganese up to 0.50
- sulfur 0.15 to 0.50
- silicon up to about 1
- phosphorus up to about 0.20
- and remainder iron except for incidental impurities and
- wherein the maximum manganese to sulfur ratio is 1 to 1.
6. The steel of claim 5 having carbon plus nitrogen up to about 0.04.
7. The steels of claims 5 or 6 having from about 0.75 to 3.00 copper.
8. The steel of claims 5 or 6 having from 1.00 to 2.50 copper.
9. Machined austenitic stainless steel fittings and articles characterized by having improved machinability and resistance to corrosion in acid soft drink syrups, especially in the passivated condition, said fittings and articles consisting essentially of, by weight percent
- carbon plus nitrogen up to about 0.05
- chromium 16 to 20
- nickel 6 to 14
- manganese up to 0.60
- sulfur 0.15 to 0.50
- silicon up to about 1

- phosphorus up to about 0.20
- molybdenum up to about 1
- and remainder iron except for incidental impurities.
10. The machined austenitic stainless steel fittings and articles of claim 9 having carbon plus nitrogen up to about 0.04.
11. The machined austenitic stainless steel fittings and articles of claims 9 or 10 having from about 0.75 to 3.00 copper.
12. The machined austenitic stainless fittings and articles of claims 9 or 10 having from 1.00 to 2.50 copper.
13. Machined austenitic stainless steel fittings and articles characterized by having improved machinability and improved resistance to corrosion in acid soft drink syrups in the passivated condition, said fittings and articles consisting essentially of, by weight percent
- carbon plus nitrogen up to about 0.05
- chromium 17 to 19
- nickel 8 to 11
- manganese up to 0.50
- sulfur 0.15 to 0.50
- silicon up to about 1
- phosphorus up to about 0.20
- molybdenum up to 1
- and remainder iron except for incidental impurities and
- wherein the maximum manganese to sulfur ratio is 1 to 1.
14. The machined austenitic stainless steel fittings and articles of claim 13 having carbon plus nitrogen up to about 0.04.
15. The machined austenitic stainless steel fittings and articles of claims 13 or 14 having from about 0.75 to 3.00 copper.
16. The machined austenitic stainless steel fittings and articles of claims 13 or 14 having 1.00 to 2.50 copper.

\* \* \* \* \*

UNITED STATES PATENT AND TRADEMARK OFFICE  
CERTIFICATE OF CORRECTION

PATENT NO. : 4,933,142

DATED : June 12, 1990

INVENTOR(S) : Walter T. HASWELL, JR., et al.

It is certified that error appears in the above-identified patent and that said Letters Patent is hereby corrected as shown below:

Claim 1, column 6, line 58, delete ", especially".

Claim 3, column 7, line 3, delete "claim 2" and insert  
--claims 1 or 2--; and after "0.75" insert --to 3.00--.

Claim 4, column 7, line 5, delete "claim 2" and insert  
--claims 1 or 2--.

Claim 5, column 7, line 9, delete ", especially".

Claim 9, column 7, line 31, delete ", especially".

Signed and Sealed this  
Eighth Day of October, 1991

*Attest:*

HARRY F. MANBECK, JR.

*Attesting Officer*

*Commissioner of Patents and Trademarks*